

C. J. CONARD,  
METHOD FOR RENEWING WORN OUT PLOW POINTS.  
APPLICATION FILED MAR. 22, 1916.

1,241,094.

Patented Sept. 25, 1917.

Fig. 1.



Fig. 2.



Fig. 6.



Fig. 7.



Fig. 5.



C. J. Conard <sup>Inventor</sup>

Witnesses

Philip G. Mull  
Francis S. Dowell

By

D. Swift & Co  
*113* <sup>113</sup> Attorneys

# UNITED STATES PATENT OFFICE.

CYRUS J. CONARD, OF OLNEY SPRINGS, COLORADO.

## METHOD FOR RENEWING WORN-OUT PLOW-POINTS.

1,241,094.

Specification of Letters Patent. Patented Sept. 25, 1917.

Application filed March 22, 1916. Serial No. 85,877.

*To all whom it may concern:*

Be it known that I, CYRUS J. CONARD, a citizen of the United States, residing at Olney Springs, in the county of Crowley, State of Colorado, have invented a new and useful Method for Renewing Worn-Out Plow-Points; and I do hereby declare the following to be a full, clear, and exact description of the invention, such as will enable others skilled in the art to which it appertains to make and use the same.

This invention relates to an improved method for renewing or repointing the point of a worn out plow.

15 In the drawings:—

Figure 1 is a view of a plow point and a plate in position, thereby disclosing the first step for renewing the worn out point of the plow.

20 Fig. 2 is a view disclosing the second step.

Fig. 3 is a view in side elevation showing the lug carried by the plate to be welded to the point as having been headed, which is the third step in the method for renewing a worn out plow point.

Fig. 4 is a view showing the plate to be welded to the plow point, as having been bent, which is the fourth step in renewing the worn out plow point.

30 Fig. 5 is a view of the plow point entirely renewed.

Fig. 6 is a perspective view of the plate and its lugs, to be welded to the worn out plow point.

35 Fig. 7 is a detail perspective view of a worn out plow point, illustrating the enlargement 11, which constitutes sufficient body or metal stock to which said plate may be welded, so that the plow point may be properly renewed.

Referring more especially to the drawings, 1 designates a plow point, which is provided with an opening 4, whereby the plow point may be fastened to the plow standard (not shown). The plow point or portion 5 when it becomes worn or dull may be renewed or repointed. This repointing is accomplished, by first heating the point 5 from *a* to *b* sufficiently for welding purposes, as indicated by the shade lines 6, after which a piece of malleable sheet steel 7 of suitable size and shape, preferably as shown in Figs. 1, 3 and

6 is first attached to the heated point 5, as shown in Fig. 2. This plate or piece of sheet metal 7 is provided with a spur 8 upon one of its faces, which spur is rectangular in cross section. However, the sheet metal plate 7 (which may be any desired thickness) remains cold. After heating the point to a suitable heat, the plate 7 (which remains cold) is arranged as illustrated in Fig. 1. The spur 60 8 is then driven transversely through the point 5, after which the extremity of the spur is riveted or clenched, as shown in Fig. 3. The rectangular shape of the spur 8 prevents twisting or displacement of the plate 65 7. While the plate is attached as shown in Figs. 2 and 3, the plate and the point are then brought to welding heat, after which the plate is bent as shown in dotted lines in Fig. 2, and then to the full line position in 70 Fig. 4, and subsequently completely welded to the point 5, and drawn out thereby providing a renewed plow point. In other words, a plow point, which is completely renewed, as shown at 10 in Fig. 5. The plow point 75 has a flange 3 and adjacent where said flange merges into said point 5, an enlargement 11 is provided, thereby affording sufficient stock through which the spur may be driven, and whereby the point may be welded when attaching the plate 7.

The invention having been set forth, what is claimed as new and useful is:—

The method herein described of renewing the point of a worn out plow, consisting in 85 applying to one side of the worn point a plate of suitable size and shape and having a spur adjacent one edge thereof, driving said spur entirely through the plow point, heading the projecting end thereof, bending 90 the plate around the worn point, heating the whole to a welding heat, and then welding the whole together, by percussive blows, and simultaneously drawing out the metal of the plate to form the renewed point. 95

In testimony whereof I have signed my name to this specification in the presence of two subscribing witnesses.

CYRUS J. CONARD.

Witnesses:

BERT TABOR,  
JOSEPH M. SUMMERTALTER.